

# UNITED STATES PATENT OFFICE.

PAUL BESNIER, OF NEW ORLEANS, LOUISIANA

## PROCESS OF DYEING.

988,300.

Specification of Letters Patent.

Patented Apr. 4, 1911.

No Drawing.

Application filed July 6, 1910. Serial No. 570,656.

*To all whom it may concern:*

Be it known that I, PAUL BESNIER, of New Orleans, in the parish of Orleans and State of Louisiana, have invented certain new and useful Improvements in Processes of Dyeing; and I hereby declare that the following is a full, clear, and exact description thereof.

This invention is a novel improvement in the art of dyeing fabrics—particularly cotton fabrics,—and its object is to fix the colors therein during the dyeing process so that they will be fast.

The invention consists of a preparation which, when added to the dye, will act on the tissue of the fabric in such a manner as to make it take the dye and retain the color in a manner far superior to that obtained by any other process, with less handling, less rinsing, less labor, and also less dye,—thus greatly economizing both time and expense.

The invention in brief comprises a new preparation and process of using same in dyeing fabrics, and by this invention cotton fabrics can be dyed a true and fast black, and also wool and silk.

In carrying out the invention I first prepare a fixing powder composed of common salt; Glauber salt, lye, and naphthalene. These ingredients are chemically known as chlorid of sodium ( $NaCl$ ); sodium sulfate ( $Na_2SO_4 + 10H_2O$ ); carbonate of potash ( $K_2CO_3$ ); naphthalene ( $C_{10}H_8$ ). I preferably use the following proportions of these ingredients by weight: 25 parts salt, 10 parts Glauber salt, 1 part lye, 1 part naphthalene. These ingredients are mixed together, heated gently and stirred briskly, and then allowed to cool. The mixture when cold is in the form of a coarse powder.

In using the preparation I add about 40 twelve (12) ounces of the above powder to ten (10) gallons of water, and boil same, and then add the desired dye; when the dye is dissolved, I place the tissue, or fabric, to be dyed in this bath, and boil it therein for 45 about thirty minutes; then remove the tissue and rinse it in cold water. By this powder and process I can (for instance) dye cotton a true black, with little handling, and in a very short time.

This powder and process can be used for dyeing true black, not only cotton, but also wool and silk. It may also be used for fixing other colors in dyeing.

What I claim is:

1. A powder for use in the dyeing of fabrics, consisting of salt, Glauber salt, lye, and naphthalene, substantially as described.

2. The herein described powder for use in the dyeing of fabrics consisting of about 60 25 parts of salt, 10 parts of Glauber salt, 1 part of lye, and 1 part of naphthalene, substantially as described.

3. The herein described method of preparing a fixing powder for use in the dyeing of 65 fabrics consisting in mixing salt, Glauber salt, lye and naphthalene, heating same and stirring until mixed, and then allowing same to cool.

In testimony that I claim the foregoing as 70 my own, I affix my signature in presence of two witnesses.

PAUL BESNIER.

Witnesses:

F. C. PHILIPPE, Jr.,  
GUSTAVE GILLOT.